

June 30, 1925

1,544,042

J. K. SHAW

FIBER BOARD OF FELTED INTERLACED FIBERS

Filed March 26, 1920

2 Sheets-Sheet 1



Inventor

John K. Shaw, by  
T. C. Witherspoon

Attorney

June 30, 1925.

1,544,042

J. K. SHAW

FIBER BOARD OF FELTED INTERLACED FIBERS

Filed March 26, 1920

2 Sheets-Sheet 2

Fig. 2.



Fig. 4.



Fig. 3.



Fig. 5.



Inventor

John K. Shaw, by  
T. G. Witherspoon

Attorney

## UNITED STATES PATENT OFFICE.

JOHN K. SHAW, OF MINNEAPOLIS, MINNESOTA, ASSIGNOR TO C. F. DAHLBERG, OF ST. PAUL, MINNESOTA.

## FIBER BOARD OF FELTED INTERLACED FIBERS.

Application filed March 26, 1920. Serial No. 368,995.

To all whom it may concern:

Be it known that I, JOHN K. SHAW, a citizen of the United States, residing at Minneapolis, in the county of Hennepin and State of Minnesota, have invented certain new and useful Improvements in Fiber Boards of Felted Interlaced Fibers; and I do hereby declare the following to be a full, clear, and exact description of the invention, 10 such as will enable others skilled in the art to which it appertains to make and use the same.

This invention relates to fiber boards composed of felted interlaced fibers, and 15 has for its object to provide a board of this character which will be more efficient in use and less costly to manufacture than those heretofore proposed.

With these and other objects in view the 20 invention consists in the novel details of construction and combinations of parts constituting the board, all as will be more fully hereinafter disclosed and particularly pointed out in the claims.

Referring to the accompanying drawings forming a part of this specification in which like numerals designate like parts in all 25 the views:—

Figure 1 is a diagrammatic sectional view 30 of an apparatus suitable for making a fiber board in accordance with this invention;

Figure 2 is a diagrammatic view illustrating the disposition of the individual 35 fibers during the making of the board and before reaching the traveling surface;

Figure 3 is a view similar to Figure 2 illustrating the action of the traveling surface upon the individual fibers;

Figure 4 is a diagrammatic sectional view 40 of a fiber board made in accordance with this invention and before it passes the finishing rolls; and

Figure 5 is an enlarged diagrammatic view of a bagasse or analogous fiber of which 45 this board is composed.

In order that the precise invention may be the more clearly understood it is said: I am well aware that various fiber sheets and other articles have heretofore been made 50 from bagasse and similar fibers, which are by nature provided with a pithy substance, but in so far as I am aware, all of such fibers have been deprived of their pith before being manufactured into sheets, and 55 therefore, prior to this invention no one has

utilized the true felting action of these pith like protuberances on the fibers, to make a stronger and better board as is done in this case. But in order to cause a true interlocking or felting action between the fibers, special machinery is required, such as is disclosed in the drawings, and as the novel structure of this board will be best understood from a description of the operation of said machinery I will disclose the same as follows:

1 indicates any suitable tank for holding the stock consisting of water and cooked fibers, 2 the bottom of said tank, 3 an inclined false bottom located above the bottom 2, 4 a roll or drum near the lower end of said false bottom 3, 5 a plurality of supporting rolls, 6 a guide and compression roll adjustable on the slide, or other movable means 7, 8 a guide roll similar to the roll 4, and 9 a guide and tensioning roll adjustable on the means 10. Passing over the rolls just mentioned is the endless foraminous belt or surface 11, conveniently made of wire cloth, and having the oppositely moving portions or runs 12 and 13.

Between the runs 12 and 13 is located the water outlet 15, provided with the controlling means or gate 16 which may be suitably manipulated as by the handle or other device 17.

Coacting with the foraminous surface or belt 11, and in close proximity thereto as regards one portion thereof, is the foraminous belt 18, passing over and around the series of guide rolls 19, 20, 21, 22, 23 and 24. Said belt 18 also passes over the compression and guide roll 25 coacting with the compression roll 6, and adjustably mounted on the movable means 26. 27 represents a tension and guide roll, adjustably mounted on the means 28, and 29 an outlet for the water passing through the belt 18, controlled by the gate 30 and adjustable through the handle 31. 32 and 33 represent suitable water seals made of flexible material for the belts 11 and 18 respectively.

35 represents a channel or passage for water and fibers which may be maintained at any desired hydrostatic head 36, 37 an opening from the channel 35 into the tank space or chamber 38, and 39 a top or partition separating said chamber or space 38 from the remainder of the tank. 40 represents a second channel for water and pulp 41.

fibers, 41 the head thereof, 42 an opening from said channel into the tank chamber or space 43, and 44 a partition which with the partition 39 serves to separate said space 43 from the rest of the tank. 45 represents a third channel for water and fibers having a head 46, 47 an opening into the tank chamber or space 48, and 49 a partition co-acting with the partition 44 to segregate 10 said space 48 from the remainder of the tank.

The foregoing construction is, or may be the same as is described and claimed in my copending application, Serial Number 15 368990, filed March 26, 1920, Patent No. 1,532,083, dated March 31, 1925, and entitled Process of and apparatus for making fiber boards.

The operation of this machine will be 20 understood from what follows:

It is preferred to use long fibers, but of course fibers of any usual length may be employed. By reason of the direction of flow of the water through the chambers 38, 25 43 and 48, and by reason of the natural tendency of the flowing water to laterally separate said fibers, the latter will be brought into positions more or less parallel to each other, and more or less perpendicular 30 to the line of travel of the surface 13, while at the same time all of said fibers will occupy positions more or less staggered with relation to their neighbors as shown. Accordingly a large percentage of the forward 35 ends 61 of said fibers will first contact with said surface 13, and will be carried along by the belt from the positions shown in Figure 2 to those shown in Figure 3, for the rear ends 62 of said fibers will have lagged 40 behind the front ends 61, in the water, so that the front row of said fibers assume a somewhat curved or bent shape. The second row, or those fibers 63 immediately following, and which have not reached the 45 surface 13, but have reached the rear ends 63 of the fibers 60, are now forced by the oncoming water to contact at their forward ends against the curved fibers 60. And as said fibers 63, originally, due to their parallel positions as shown at 63 in Figure 2, 50 were more or less staggered or interlaced with the fibers 60 before the latter became curved, it is evident that this interlacing or entangling action between the fibers 60 and 55 63 will be enhanced or increased by the oncoming water after said curvature takes place.

It results from the actions just described 60 that said fibers 63 become themselves more or less curved, as indicated in Figure 3, due to the transverse movement of the fibers 60, and that a third row of fibers 64 which are also interlaced or staggered with the fibers 63 will become in time curved and entangled 65 with the fibers 60 and 63 that have

preceded said fibers 64. It thus results that owing to the floating of the fibers into parallel, interlaced or staggered positions, and in a direction transverse to the traveling surface 13, the entanglement of the fibers is 70 continuous between successive rows; and the pressure of the water causes the whole to be very loosely assembled in their interlaced positions on said surface, thus forming an open mass of fibers more compact 75 next to the wire than away from it. This mass is carried through the opening 70 into the space 43, with one or more partially curved and partially entangled layers similar to the fibers 60 and 63 clinging to it. 80

In said chamber or space 43, other fibers similar to the fibers 64 become interlaced and entangled with the layers on the belt, and the process of entanglement and massing proceeds as before. In the meantime 85 layers of fibers in all respects similar to the layers 60, 63 and 64 are interlaced, entangled and massed on the traveling belt 18 from the space or chamber 48. This second mass of fibers are carried through the opening 71 90 by the belt 18 in a condition similar to the first mentioned mass that passes the opening 70, and the fibers in the space 43 interlace, and become entangled with said second mass in a manner similar to that described 95 in connection with said first mentioned mass. The result is, owing to these parallel and staggered relations, the fibers in the space 43 constitute a third mass of fibers which are interlaced and entangled with 100 each other, as well as with each of said first named masses.

As a result of the foregoing entanglements of the various fibers and the motion of the surfaces 13 and 18, the mass of fibers are carried through the opening 75, 105 between the compression or compacting rolls 6 and 25, and is formed into the sheet or board 76, all as will be readily understood.

An important feature of this invention resides not only in being able to thus interlace, or entangle, the fibers in the body of the sheet, but also in being able to vary the kind, size, and class, of fibers in different portions of the sheet. That is to say, I may feed to the channel 35, one kind of fibers, 110 which may be relatively short or more expensive fibers than are those fed to the channel 40, and I may feed to the channel 45, the same class of fibers as are fed to the channel 35, or I may feed a totally different class of fibers. In other words I may provide as many channels 35, 40 and 45, as 115 there are different characters of fibers in the finished board, and I may place in the first channel 35 and in the last channel 45 any characters of fibers I desire, whereupon the board will be provided with an outer layer 77 corresponding to the fibers that are fed to the channel 35, with another outer layer 120 125 130

78 corresponding to the fibers that are fed to the channel 45, and with one or more intermediate layers 79 corresponding to the character of the fibers which are fed to the channel 40 and to any other channels which may be located intermediate of the channels 35 and 45.

In making this board I prefer to use bagasse and other pith carrying fibers such as those from cane, bamboo, sorghum, etc., and which have been treated according to the process disclosed and claimed in my co-pending application, Serial Number 368993 filed March 26, 1920, Patent No. 1,501,925 dated July 22, 1924, and entitled Bagasse fiber and process of producing the same. In brief such process which consists in dissolving out the binding material between the fibers as well as the brittle material encasing the fibers, without impairing the original strength of the fibers, and, also, without depriving the individual fibers of their pith like protuberances, or knots, which are so valuable as a felting agency as well as for use as a heat insulating means. Further by controlling the action in the heating engine, and the strength of the dissolving solution, the size of the bundles of fibers can be controlled, and therefore the heat insulating.

It therefore follows that when the fibers provided with the pith like protuberances 100 and the hook like portions 101 are interlaced in the manner disclosed, they become so firmly interlocked that this felting action resembles that of wool more nearly than it does the so called felting of cotton and wood fibers. So pronounced is this difference of structure that actual tests have shown that a fiber board constructed as above disclosed, and only loosely compacted, so as to include a large number of air cells to serve as a heat insulating medium, is very much stronger both as to tensile strength and breaking strength than is a similar board made from wood, flax or other fibers. In other words, even when this board is subjected to transverse breaking strains the hook like portions and the pith like projections on the individual fibers interlock and thus prevent the fibers from slipping over each other, with the result that a large number of the fibers are strained longitudinally instead of transversely of their length and thus is the strength of the board very greatly increased.

But the greatest difference between this board and the prior boards appears when the fibers are compacted with a heavy pressure of say 400 lbs. to the square inch. Such a pressure produces a board which is hard and resilient like wood. In fact it may be whittled, sawed and nailed like wood and constitutes a valuable substitute for the higher grades of lumber for the manufacture of trunks, furniture, etc. Actual tests

have shown it to possess a tensile strength of over 16,000 pounds while wood fiber, flax fiber and other boards of a similar size and make only showed a tensile strength of about 1100 pounds. In the same way my bagasse board showed a transverse breaking strength of 285 pounds while the other boards showed a breaking strength of only 113 pounds.

In producing the board on the machine illustrated, I further prefer to permit a very large proportion of the water, say 90% of the same to escape through the opening 15, while a very much smaller proportion, say 10% escapes through the opening 29. The gates 16 and 30 are conveniently manipulated to effect this division of the water, while maintaining the desired proper steady flow through the surfaces 13 and 18 to produce the desired results. But of course the proportions of water that escape through the two openings mentioned may be widely varied according to the results sought in the finished board.

The rolls 6 and 25 are readily adjusted by the means illustrated to produce any desired compression in the openings 75 between said rolls, so that the fiber board may be given any desired degree of porosity. In fact, by using relatively large fibers in the channel 40, and relatively fine fibers in the channels 35 and 45, I am enabled to control the air spaces in the body of the board, and thereby to control its heat-insulating qualities.

The heads 36, 41 and 46 of the liquid in the channels 35, 40 and 45 are so maintained that there will be a minimum tendency of liquid to flow between the chambers or spaces 38, 43 and 48. In other words, the pressures of the liquid in the last mentioned chambers are maintained as nearly equal as possible, and thus a minimum tendency of the fibers to mix in the said spaces is secured.

The interlacing process is facilitated by the fact that the openings 37, 42 and 47 are of a less area than are the spaces 38, 43 and 38 into which the fibers are led. In other words the fibers must first pass through the openings at a relatively high velocity and close relation to each other; and they are then immediately released into a wider space where they take on a lesser velocity, and naturally spread out as they pass along with the water, thus assuming the parallel relations indicated in Figure 2.

It will now be clear that my board is composed of different layers of interlaced pith carrying fibers which produce not only a true felting, or entangling action, but, also, high heat insulating qualities owing to the pith particles being largely composed of closed air cells. So great are the advantages of these pith like protuberances that I find that an excellent product can be produced

with other fibers so long as say 20% or more of the board consists of these said pith carrying fibers.

It is obvious that those skilled in the art <sup>5</sup> may vary the details of the invention without departing from the spirit thereof, and therefore I do not wish to be limited to the above disclosure except as may be required by the claims.

10. What I claim is:—

1. The herein described fiber board composed of different masses of different kinds of fibers, a portion of the fibers of each of said masses interlaced with a portion of the <sup>15</sup> fibers of an adjacent mass, and a portion of said fibers carrying natural pith like protuberances serving as entangling agents between the fibers.

2. The herein described fiber board composed of different masses of different kinds of fibers, a portion of the fibers of one mass being interlaced with a portion of the fibers of an adjacent mass, and more than twenty <sup>25</sup> per cent of said fibers carrying natural pith like protuberances serving as inter-entangling means between the fibers.

3. The herein described fiber board composed of different masses of different kinds of pith carrying fibers interlaced with each <sup>30</sup> other, said fibers carrying their pith in the

form of protuberances attached to the individual fibers which offer resistance when one fiber tends to slip over another fiber.

4. The herein described fiber board composed of different masses some of which are <sup>35</sup> pith carrying bagasse fibers interlaced with each other, said fibers carrying their pith in the form of protuberances attached to the individual fibers which offer resistance when one fiber tends to slip over another fiber, <sup>40</sup> and one mass of said fibers being of a quality different from another mass.

5. The herein described heat insulating fiber board composed of different masses one of which is composed of bagasse fibers carrying its natural pith, the fibers of adjacent <sup>45</sup> masses interlaced with each other, and one of said masses composed of larger aggregates of fibers than another mass in order to provide larger air cells between the masses.

6. The herein described fiber board devoid of a peeling structure and composed of different masses of bagasse fibers interlaced with each other and carrying their natural pith, said fibers and masses being highly <sup>50</sup> compressed together to form a board of a high tensile and breaking strength for use as a substitute for lumber.

In testimony whereof I affix my signature.

JOHN K. SHAW.